# EUROPEAN PATENT SPECIFICATION

(11) **EP 0 461 523 B1**
(45) Date of publication and mention of the grant of the patent: **20.11.2002**
(21) Application number: 91109105.6
(22) Date of filing: 04.06.1991
(51) Int. Cl.: G03G 5/06

(54) **Photoconductive imaging members with titanium phthalocyanine**
Photoleitfähiges Abbildungselement mit Titanyl-Phthalocyaninen
Elément photoconducteur à base de titanium de phtalocyanine

(30) Priority: 14.06.1990 US 537714
(43) Date of publication of application: 18.12.1991
(73) Proprietor: XEROX CORPORATION, Rochester New York 14644 (US)
(72) Inventor: Hor, Ah-Mee, Mississauge, Ontario, L5L 5B1 (CA); Duff, James M., Mississauga, Ontario, L5N 2E8 (CA); Allen, Charles G., Toronto, Ontario, M6P 1J3 (CA); Mayo, James D., Toronto, Ontario, M6P 2S4 (CA)
(74) Representative: Grünecker, Kinkeldey, Stockmair & Schwanhäusser Anwaltssozietät

(56) References cited:
- EP-A- 0 314 100
- US-A- 4 882 254
- 5. INTERNATIONAL CONGRESS ON ADVANCES IN NONIMPACT PRINTING TECHNOLOGIES, November 1989, SAN DIEGO CALIFORNIA US, pages 37-42, Y. FUJIMAKI ET AL.: "NEAR-INFRARED SENSITIVE ELECTROPHOTGRAPHIC PHOTOCONDUCTORS USING PHTHAOLOCYANINE"
- DATABASE WPIL, no.90-19561, Derwent Publications && JP-A-1299874 (Toyo Ink MFG K. K.) 04-12-1989
- JOURNAL OF IMAGING SCIENCE. vol. 34, no. 6, December 1990, SPRINGFIELD US pages 234 - 242; T. ENOKIDA ET AL.: "POLYMORPHS OF OXOTITANIUM PHTHALOCYANINE AND THEIR APPLICATIONS FOR PHOTORECEPTORS"

## Description

This invention is generally directed to photoresponsive imaging members, and more specifically the present invention is directed to layered photoconductive members comprised of a specific γ-titanyl phthalocyanine (TiOPc) as charge generating material. The present invention envisions the selection of specific titanyl phthalocyanine pigments as organic photogenerator materials in photoresponsive imaging members containing a charge transport layer comprised of aryl amine hole transport molecules. The aforementioned photoresponsive imaging members can be negatively charged. The layered photoconductor imaging members of the present invention can be selected for a number of different known imaging and printing processes including, for example, electrophotographic imaging processes, especially xerographic processes wherein charged images are rendered visible with toner compositions. Generally the imaging members of the present invention are sensitive in the wavelength regions of from 500 to 900 nanometers. In an embodiment of the present invention the imaging members thereof have stable charging and excellent photosensitivity or photoconductive properties in the wavelength range of, for example, from 600 to 850 nanometers. Accordingly, these imaging members are particularly .suitable for selection in the electronic printer processes wherein e.g. light emitting diodes (LED), helium-neon gas lasers of DAAS diode lasers can be selected as the imaging light sources.

There is disclosed in U.S. Patent 4,898,799 a photoreceptor with a specific carrier transporting substance and a titanyl phthalocyanine which has major peaks as indicated, reference for example Claim 3, and this phthalocyanine, it is believed, has a maximum optical absorption peak, that is the maximum wavelength of the absorption spectrum is at about 817 nanometers, which is a different titanium phthalocyanine than that initially used in the present invention which has optical absorption peaks at 660 and 750 nanometers as determined, for example, by a spectrometer. In U.S. Patent 4,882,427 there is disclosed (1) an optical semiconductor material comprising a noncrystalline titanium phthalocyanine compound, which does not show substantial x-ray diffraction peak in an x-ray diffraction chart, (2) a pseudo noncrystalline titanium phthalocyanine compound with broad x-ray diffraction peaks at certain Bragg angles and (3) an assembly of said noncrystalline titanium phthalocyanine compound, reference the Abstract of the Disclosure for example. A number of Japanese Laid Open Publications relate to titanyl phthalocyanine including 64-17066, laid open January 20, 1989, directed to a light sensitive material containing titanyl phthalocyanine of which the principle peak of the Bragg angle is as indicated, and it is further disclosed in this Laid Open Publication that the alpha-type of titanium phthalocyanine as illustrated in Japanese 61-239248 is unsatisfactory in the sensitivity and the electrical potential stability when repeatedly used, the titanyl phthalocyanine of this publication being of the structure as illustrated on page 8 and a method for producing the titanyl phthalocyanine illustrated on page 9 wherein, for example, titanyl tetrachloride and phthyl dinitrile are reacted in chloronaphthalene as a solvent to provide dichloro titanyl phthalocyanine, which is subjected to hydrolysis to result in the alpha-type titanyl phthalocyanine, and this is preferably treated with an electron releasing solvent such as 2-ethyl ethoxy ethanol; Japanese Laid Open 20365, January 28, 1988, directed to novel titanyl phthalocyanine crystals whose x-ray diffraction pattern evidences a diffraction angle of 27.3°C characterized in that an aromatic hydrocarbon solvent is added to an aqueous suspension of type alpha titanium phthalocyanine and the mixture is heated, note the disclosure beginning on page 3; Japanese Laid Open 171771, August 2, 1986, which discloses a method to purify metallo phthalocyanines characterized in that these phthalocyanines are purified by a N-methyl pyrrolidone treatment, which is usually carried out by heating at a temperature of from 130 to 180°C; Japanese Laid Open 256865/1987 directed to the method for the preparation of oxytitanium phthalocyanines by condensing phthalodinitrile with titanium tetrachloride and organic solvent at 170°C to 300°C and subsequently by hydrolyzing the resulting contact condensate, heating the organic solvent to a temperature of from 160 to 300° in advance, reference for example what appears to be the first claim; and Japanese Laid Open Publications 256866, November 9, 1987; 256867, November 9, 1987; 120564, May 12, 1989; and Japanese Application 278937, published May 12, 1989, directed to an electrophotographic photosensitive material wherein the charge generating layer consists of an oxytitanyl phthalocyanine.

Layered photoresponsive imaging members are described in a number of U.S. patents, such as U.S. Patent 4,265,900, wherein there is illustrated an imaging member comprised of a photogenerating layer, and an aryl amine hole transport layer. Examples of photogenerating layer components include trigonal selenium, metal phthalocyanines, vanadyl phthalocyanines, and metal free phthalocyanines. Additionally, there is described in U.S. Patent 3,121,006 a composite xerographic photoconductive member comprised of finely divided particles of a photoconductive inorganic compound dispersed in an electrically insulating organic resin binder. The binder materials disclosed in the '006 patent comprise a material which is incapable of transporting for any significant distance injected charge carriers generated by the photoconductive particles.

Many other patents are in existence describing photoresponsive devices including layered devices containing generating substances, such as U.S. Patent 3,041,167, which discloses an overcoated imaging member with a conductive substrate, a photoconductive layer, and an overcoating layer of an electrically insulating polymeric material. This member is utilized in an electrophotographic copying method by, for example, initially charging the member with an electrostatic charge of a first polarity, and imagewise exposing to form an electrostatic latent image which can be subsequently developed to form a visible image. Prior to each succeeding imaging cycle, the imaging member can be charged with an electrostatic charge of a second polarity, which is opposite in polarity to the first polarity. Sufficient additional charges of the second polarity are applied so as to create across the member a net electrical field of the second polarity. Simultaneously, mobile charges of the first polarity are created in the photoconductive layer such as by applying an electrical potential to the conductive substrate. The imaging potential which is developed to form the visible image is present across the photoconductive layer and the overcoating layer.

Photoresponsive imaging members with squaraine photogenerating pigments are also known, reference U.S. Patent 4,415,639. In this patent there is illustrated a photoresponsive imaging member with a substrate, a hole blocking layer, an optional adhesive interface layer, an organic photogenerating layer, a photoconductive composition capable of enhancing or reducing the intrinsic properties of the photogenerating layer, and a hole transport layer. As photoconductive compositions for the aforementioned member there can be selected various squaraine pigments, including hydroxy squaraine compositions. Moreover, there is disclosed in U.S. Patent 3,824,099 certain photosensitive hydroxy squaraine compositions. According to the disclosure of this patent, the squaraine compositions are photosensitive in normal electrostatographic imaging processes.

The use of selected perylene pigments as photoconductive substances is also known. There is thus described in Hoechst European Patent Publication 0040402, DE3019326, filed May 21, 1980, the use of N,N'-disubstituted perylene-3,4,9,10-tetracarboxyldiimide pigments as photoconductive substances. Specifically, there is disclosed in this publication evaporated N,N'-bis(3-methoxypropyl)perylene-3,4,9,10-tetracarboxyldiimide dual layered negatively charged photoreceptors with improved spectral response in the wavelength region of 400 to 700 nanometers. A similar disclosure is revealed in Ernst Gunther Schlosser, *Journal* of *Applied Photographic Engineering,* Vol. 4, No. 3, page 118 (1978). There is also disclosed in U.S. Patent 3,871,882 photoconductive substances comprised of specific perylene-3,4,9,10-tetracarboxylic acid derivative dyestuffs. In accordance with the teachings of this patent, the photoconductive layer is preferably formed by vapor depositing the dyestuff in a vacuum. Also, there is specifically disclosed in this patent dual layer photoreceptors with perylene-3,4,9,10-tetracarboxylic acid diimide derivatives, which have spectral response in the wavelength region of from 400 to 600 nanometers. Also, in U.S. Patent 4,555,463, there is illustrated a layered imaging member with a chloroindinium phthalocyanine photogenerating layer. In U.S. Patent 4,587,189, there is illustrated a layered imaging member with a perylene pigment photogenerating component. Both of the aforementioned patents disclose an aryl amine component as a hole transport layer.

Furthermore, there is disclosed in U.S. Patent 4,419,427 electrographic recording mediums with a photosemiconductive double layer comprised of a first layer containing charge carrier perylene diimide producing dyes, and a second layer with one or more compounds which are charge transporting materials when exposed to light, reference the disclosure in column 2, beginning at line 20. Also of interest with respect to this patent is the background information included in columns 1 and 2, wherein perylene dyes of the formula illustrated are presented.

Additionally, there are illustrated in U.S. Patent 4,429,029 electrophotographic recording members with perylene charge carrier producing dyes and a charge carrier aryl diamine transporting layer.

With the photoresponsive imaging members of the present invention, the photogenerating titanyl phthalocyanine layers are prepared by vacuum deposition enabling superior image quality in comparison to the binder or binderless dispersed layers obtained by the spray coating or solution casting techniques as illustrated in the '029 patent. Vacuum deposition enables, for example, layers of uniform thickness and substantial smoothness as contrasted to layers of ununiform thickness and surface roughness with binder or binderless dispersed layers prepared by spray coating processes; very thin layers of 0.1 µm (micron) or less are permitted whereas with binder or binderless dispersed layers, thicknesses are generally about 0.5 µm (micron) or more; and continuous layers with no large voids or holes result, while dispersed layers usually contain holes or voids thereby adversely affecting image resolution.

Furthermore, with the imaging members of the present invention comprised of the vacuum deposited gamma titanyl phthalocyanines and aryl amine hole transporting compounds superior xerographic performance occurs as low dark decay characteristics result and higher photosensitivity is generated, particularly in comparison to several prior art imaging members prepared by solution coating or spray coating, reference for example U.S. Patent 4,429,029 mentioned hereinbefore.

In a patentability search report, the following U.S. patents were listed: 4,882,427, see columns 3 and 9, for example; 4,536,461 wherein a vacuum evaporated metal free phthalocyanine is selected; 4,701,396 and 4,898,799 disclose certain titanyl phthalocyanines as photogenerators; 4,471,039; 4,546,059; 4,555,463; 4,557,989; 4,582,772; 4,587,189; 4,731,312 and 4,732,832.

While the above-described photoresponsive imaging members are suitable for their intended purposes, there continues to be a need for improved members, particularly layered members, having incorporated therein specific phthalocyanine pigment compositions and aryl amine hole transport compounds. Additionally, there continues to be a need for layered imaging members comprised of specific aryl amine charge transport compositions, and as photogenerating materials titanyl phthalocyanine pigments with acceptable photosensitivity, low dark decay characteristics, high charge acceptance values, and wherein these members can be used for a number of imaging cycles in a xerographic imaging or printing apparatus. Furthermore, there continues to be a need for photoresponsive imaging members which can be negatively charged thus permitting the development of images, including color images, with positively charged toner compositions. Moreover, there continues to be a need for disposable imaging members with nontoxic organic pigments. Also, there is a need for disposable imaging members useful in xerographic imaging processes and xerographic printing systems wherein, for example, light emitting diodes (LED), diode lasers, helium cadmium, or helium neon lasers are selected; and wherein these members are particularly sensitive to the infrared region of the spectrum, that is, from 600 to 850 nanometers. In copending application US.Ser.No. 533 261 (D/90087 - not yet assigned), there is disclosed, for example, a process for the preparation of titanyl phthalocyanine which comprises dissolving a titanyl phthalocyanine in a solution of trifluoroacetic acid and methylene chloride; adding the resultant solution to a solvent system that will enable precipitation; and separating the desired titanyl phthalocyanine from the solution followed by an optional washing.

In copending application U.S. Serial No. (D/90244 - not yet assigned), there is disclosed, for example, a process for the preparation of phthalocyanine composites which comprises adding a metal free phthalocyanine, a metal phthalocyanine, a metalloxy phthalocyanine or mixtures thereof to a solution of trifluoroacetic acid and a monohaloalkane; adding to the resulting mixture a titanyl phthalocyanine; adding the resulting solution to a mixture that will enable precipitation of said composite; and recovering the phthalocyanine composite precipitated product.

In copending application U.S. Serial No. (D/90190 - not yet assigned), there is disclosed, for example, a process which comprises adding a pigment to a solution of trihaloacetic acid and toluene; adding the solution to a nonsolvent for the pigment; and separating the product from the solution.

"The 5th International Congress on advances in non-impact printing technologies", November 12-17, 1989, San Diego, California, US, pages 37-42: "Near-infrared sensitive electrophotographic photoconductors using oxotitanium Phthalocyanine", Y. Fujimaki, discloses an electrophotographic photoconductor containing a gamma-TiOPc polymorph having a strong absorption maximum at 850 nm.

European Patent Publication 0314100 discloses an electrophotographic sensitive material comprising a substrate, a photogenerating layer and a charge transporting layer, the photogenerating layer containing a mixture of phthalocyanine pigments comprising an alpha-TiOPc and a metal-free TiOPc.

JP-A-1299874 discloses an electrophotographic device comprising an alpha-type titanyl phthalocyanine as charge-generating agent and a styryl compound as charge-transferring agent.

It is an object of the present invention to provide photoconductive imaging members which are substantially inert to the users thereof.

It is yet another object of the present invention to provide disposable layered photoresponsive imaging members.

A further specific object of the present invention resides in the provision of an improved photoresponsive imaging member with an aryl amine hole transport layer, and a photogenerator layer comprised of specific phthalocyanine pigment compositions.

In yet another specific object of the present invention there are provided negatively charged layered photoresponsive imaging members comprised of vacuum evaporated titanyl phthalocyanine (TiOPc) pigment compositions optionally dispersed in a resinous binder, and a hole transport layer comprised of aryl amine molecules.

It is still another object of the present invention to provide improved imaging members sensitive to light in the infrared region of the spectrum, that is from 600 to 850 nanometers.

It is yet another object of the present invention to provide imaging and printing methods with the improved photoresponsive imaging members illustrated herein.

The above objects of the present invention are solved by providing a photoresponsive imaging member comprised of a supporting substrate, a charge generating layer deposited thereon consisting of a vacuum evaporated photogenerator layer of gamma titanyl phthalocyanine of the formula C₃₂H₁₆N₈OTi with two major optical absorption peaks at 660 and 760 nm, and a charge transporting layer deposited on said charge generating layer, wherein the peaks are achieved subsequent to the deposition of said transport layer on said titanyl phthalocyanine layer, wherein the charge transport layer is an aryl amine hole transport layer comprised of molecules of the formula wherein X is selected from the group consisting of halogen and alkyl, dispersed in a resinous binder under the addition of an organic solvent, and wherein the solvent is selected from the group consisting of methylene chloride, chlorobenzene, toluene, cyclohexanone and alcohols; and
a method of imaging or printing which comprises forming an electrostatic latent image on a photoresponsive imaging member as defined above accomplishing development thereof with toner particles; subsequently transferring the developed image to a suitable substrate; and permanently affixing the image thereto.

Specific embodiments of the present invention are set forth in the attached dependent claims.

According to the present invention, there is provided a layered imaging member comprised of a photogenerating layer of gamma titanyl phthalocyanine, which phthalocyanine has a maximum wavelength of the absorption spectra or optical absorption peaks at 660 and 760 nanometers as determined by a spectrometer, which phthalocyanine is believed to be a new form of titanyl phthalocyanine, and wherein the imaging member is obtained by vacuum evaporation followed by a solution coating of an aryl amine transport layer. Although not desired to be limited by theory, it is believed that the new polymorph of the gamma form of titanyl phthalocyanine is formed by the specific solvents selected for accomplishing the coating of the transport layer including methylene chloride, chlorobenzene, toluene, cyclohexanone, and alcohols such as methanol. Thereafter, the resulting imaging member is dried, for example, by heating at a temperature in an embodiment of the present invention of from 100 to 150°C enabling the removal of any excess solvent.

As indicated before, the use of certain titanyl phthalocyanines as photogenerating layers is known, however, much of this prior art is related to the selection of pigment dispersions of certain titanyl phthalocyanines and suitable polymeric binders after the phthalocyanine pigment has been subjected to a complex and time consuming process, which is essential, it is believed, to obtain the polymorph form disclosed. For example, in U.S. Patent 4,728,592 there is illustrated the preparation of alpha-type titanium phthalocyanine polymorphs from the reaction of titanium tetrachloride and phthalonitrile followed by milling to convert the resulting titanyl phthalocyanine into particles which are then selected for forming the pigment binder dispersion. This titanium phthalocyanine exhibits typical absorption peaks at 640 and 830 nanometers as illustrated in the aforementioned patent. Also, U.S. Patent 4,898,799 specifically teaches a process in which alpha-type phthalocyanine is agitated at 50 to 180°C to convert this phthalocyanine to a polymorph with an obstacle absorption maximum peak at 817 nanometers. In addition to various complicated processes needed for obtaining special polymorph of TiOPc in small particle sizes, the preparation of stable polymeric dispersions of pigment suitable for coating is not easily attained. Pigment particles tend to grow into large particles or agglomerate to form large aggregates which either flocculate or precipitate out as sediment and hence causing great difficulties in coating smooth and uniform photogenerator layers.

In Japan Kokai Patent Application 278937 (1987), vacuum evaporated TiOPc is subjected to a treatment by immersing the evaporated film in alcohol at 25 to 40°C for 1 to 10 seconds in order to achieve the desired polymorph with absorption peaks at 700 and 790 nanometers, which is claimed to possess an improved photosensitivity. However, the process poses certain disavantages such as additional cost in the production and risks of contaminating and introducing defects in the TiOPc generator layer. Defects in the photogenerator layer generally cause print quality problems in the finished imaging members.

With the present invention, the initial titanyl phthalocyanine selected is an alpha titanyl phthalocyanine with optical absorption peaks at 660 and 750 nanometers which may be obtained or prepared by conventional methods, reference F.H. Moser and A.L. Thomas in *The Phthalocyanines, Volumes I* & *II,* CRC Press Inc., Florida, 1983. In one embodiment, the titanyl phthalocyanines are prepared by reacting phthalonitrile or 1,3-diiminoisoindoline with titanium tetrachloride or titanium tetra-alkoxide in high boiling solvents such as quinoline, chloronaphthalene, or N-methylpyrrolidone. The reaction mixture is heated to the reflux temperature of the solvent from two to 20 hours. The dark blue phthalocyanine solid formed was isolated from the reaction mixture by filtration and thoroughly washed with solvents such as e.g. dimethylformide (DMF) or alcohols. Acid dissolution process is commonly used to further purify the crude phthalocyanine obtained by first dissolving it in acids such as sulfuric acid and then diluting the acid solution in a large quantity of water or any suitable solvent mixture in which finely divided phthalocyanine particles were precipitated. Thereafter, this titanium phthalocyanine is converted to the new polymorph form gamma phthalocyanine with absorption peaks at 660 and 760 nanometers during preparation of the layered imaging member, and more specifically when the charge transport layer with solvents therein are applied to a photogenerating layer or alternatively by initially treating the formed titanium phthalocyanine with charge and specifically hole transport materials contained in a solvent.

Numerous different layered photoresponsive imaging members with the phthalocyanine pigments illustrated herein can be fabricated. In one embodiment, thus the layered photoresponsive imaging members are comprised of a supporting substrate, a charge transport layer being an aryl amine hole transport layer, and situated therebetween a vacuum evaporated photogenerator layer comprised of the vacuum evaporated titanyl phthalocyanine pigments illustrated herein. Moreover, there is provided in accordance with the present invention an improved negatively charged photoresponsive imaging member comprised of a supporting substrate, a thin adhesive layer, a titanyl phthalocyanine photogenerator vacuum evaporated layer optionally dispersed in a polymeric resinous binder, and as a top layer aryl amine hole transporting molecules dispersed in a polymeric resinous binder.

The photoresponsive imaging members of the present invention can be prepared by a number of methods, the process parameters being dependent on the member desired. Thus, these imaging members are prepared by vacuum deposition of the photogenerator layer on a supporting substrate with an adhesive layer thereon, and subsequently depositing by solution coating the hole transport layer. Deposition of the titanyl phthalocyanine is preferably accomplished in vacuum coaters operating at a pressure of (2,33 x 10⁻³ to 2,33 x 10⁻¹⁰ MPa) (10⁻⁴ to 10⁻⁶ Torr). In one embodiment, the starting material TiOPc is loaded into a crucible whose temperature is raised to 300 to 550°C to effect the sublimation of TiOPc. The sublimed vapor is then deposited onto suitable substrates situated above the crucible. Substrates can be conductive drums in rotating motion or a continuously moving metallized plastic web. The thickness of the deposited photogenerator layer is preferably selected in the range of 0.05 to 1.0 µm (micron). For the drums, the desired thickness of the TiOPc layer can be obtained by adjusting both the duration and rate of sublimation, whereas for the web, it is more conveniently achieved by controlling the sublimation rate and the speed of moving web. The vacuum evaporated TiOPc photogenerator layer is then overcoated with the charge transport layer solution which contains certain organic solvents capable of causing a desired polymorphic change in the vacuum deposited TiOPc. The resulting polymorphic change in the converted TiOPc layer produces a new optical absorption spectrum with peaks at 660 and 760 nanometers, and consequently can lead to a higher photoactivity in the infrared region. Organic solvents are selected from methylene chloride, chlorobenzene, toluene, cyclohexanone, and alcohols. Following the coating of the transport layer, the imaging members thus formed are dried at 100 to 150°C for 2 to 60 minutes to allow the removal of excess solvent.

Imaging members with the titanyl phthalocyanine pigments used in the present invention are useful in various electrostatographic imaging and printing systems, particularly those conventionally known as xerographic processes. Specifically, the imaging members of the present invention are useful in xerographic imaging processes wherein the TiOPC pigments absorb light of a wavelength of from 600 nanometers to 850 nanometers. In these known processes, electrostatic latent images are initially formed on the imaging member followed by development, and thereafter transfering the image to a suitable substrate.

Moreover, the imaging members of the present invention can be selected for electronic printing processes with gallium arsenide light emitting diodes (LED) arrays which typically function at wavelengths of 660 nanometers.

For a better understanding of the present invention and further features thereof, reference is made to the following detailed description of various preferred embodiments wherein:
Figure 1 is a partially schematic cross-sectional view of a negatively charged photoresponsive imaging member of the present invention; and
Figures 2A and 2B illustrate the absorption spectra of vacuum evaporated TiOPc prior to (A), and subsequent to (B) providing an overcoat of the specific aryl amine transport layer.

Illustrated in Figure 1 is a negatively charged photoresponsive imaging member of the present invention comprised of a substrate 1, an adhesive layer 2, a vacuum evaporated photogenerator layer 3 comprised of gamma titanyl phthalocyanine with optical absorption peaks at 660 and 760 nanometers and a hole transport layer 5 comprised of e.g. N,N'-diphenyl-N,N'-bis(3-methylphenyl)-1,1'-biphenyl-4,4'-diamine dispersed in *e.g.* a polycarbonate resinous binder 7.

Illustrated in Figure 2 are the optical absorption spectra of vacuum evaporated TiOPc film before(A)and after(B), the coating of the aryl amine transport layer of Figure 1, which coating was accomplished in methylene chloride followed by drying with heating at about 130°C for about 30 minutes. Line A is obtained for the as-evaporated film prior to any treatment and exhibits a peak at 750 nanometers. After being overcoated with the transport layer, the evaporated TiOPc film undergoes certain change to form a new polymorph whose optical spectrum (line B) evidences two characteristic peaks at 660 and 760 nanometers.

Substrate layers selected for the imaging members of the present invention can be opaque or substantially transparent, and may comprise any suitable material having the requisite mechanical properties. Thus, the substrate may comprise a layer of insulating material including inorganic or organic polymeric materials, such as Mylar a commercially available polymer; Mylar containing titanium; a layer of an organic or inorganic material having a semiconductive surface layer such as indium tin oxide, or aluminum arranged thereon, or a conductive material inclusive of aluminum, chromium, nickel, brass or the like. The substrate may be flexible or rigid and many have a number of many different configurations, such as, for example a plate, a cylindrical drum, a scroll or an endless flexible belt. Preferably, the substrate is in the form of a seamless flexible belt. In some situations, it may be desirable to coat on the back of the substrate, particularly when the substrate is a flexible organic polymeric material, an anti-curl layer, such as for example polycarbonate materials commercially available as Makrolon.

The thickness of the substrate layer depends on many factors, including economical considerations, thus this layer may be of substantial thickness, for example, over 3,000 µm (microns); or of minimum thickness providing there are no adverse effects on the system. In one preferred embodiment, the thickness of this layer is from 75 µm (microns) to 300 µm (microns).

With further regard to the imaging members of the present invention, the photogenerator layer is preferably comprised of 100 percent of the vacuum evaporated titanyl phthalocyanine pigments disclosed herein, which pigments may be optionally dispersed in resinous binders. Generally, the thickness of the photogenerator layer depends on a number of factors including the thicknesses of the other layers, and the amount of photogenerator material contained in this layer. Accordingly, this layer can be of a thickness of from 0.05 µm (micron) to 10 µm (microns) when the titanyl phthalocyanine photogenerator composition is present in an amount of from 5 percent to 100 percent by volume. Preferably, this layer is of a thickness of from 0.25 µm (micron) to 1 µm (micron) when the photogenerator composition is present in this layer in an amount of 30 percent by volume. In one very specific preferred embodiment, the vacuum deposited photogenerating layers are of a thickness of from 0.05 µm (micron) to 2 µm (microns), and preferably from 0.05 to 1.0 µm (micron). The maximum thickness of this layer is dependent primarily upon factors such as photosensitivity, electrical properties and mechanical considerations.

Illustrative examples of polymeric binder resinous materials that can be selected for the photogenerator pigment include e.g. those polymers as disclosed in U.S. Patent 3,121,006, polyesters, polyvinyl butyral, Formvar®, polycarbonate resins, polyvinyl carbazole, epoxy resins, phenoxy resins, especially the commercially available poly(hydroxyether) resins.

As adhesives there can be selected various known substances inclusive of polyesters, polyvinyl butyral, polyvinyl pyrrolidone, polyurethane, polyamide and polycarbonate. This layer is of a thickness of from 0.05 µm (micron) to 1 µm (micron).

Aryl amines selected for the hole transporting layer which generally is of a thickness of from 5 µm (microns) to 75 µm (microns), and preferably of a thickness of from 10 µm (microns) to 40 µm (microns), are molecules of the following formula: dispersed in a highly insulating and transparent organic resinous binder wherein X is an alkyl group or a halogen atom, especially those substituents selected from the group consisting of (ortho) CH₃, (para) CH₃, (ortho) Cl, (meta) Cl, and (para) Cl.

Examples of specific aryl amines are N,N'-diphenyl-N,N'-bis(alkylphenyl)-1,1-biphenyl-4,4'-diamine wherein alkyl is selected from the group consisting of ethyl such as 2-methyl, 3-methyl and 4-methyl, ethyl, propyl, butyl and hexyl. With chloro substitution, the amine is N,N'-diphenyl-N,N'-bis(halo phenyl)-1,1'-biphenyl-4,4'-diamine wherein halo is 2-chloro, 3-chloro or 4-chloro. Other hole transport molecules may be selected.

Examples of the highly insulating and transparent resinous material or inactive binder resinous material for the transport layers include materials such as those described in U.S. Patent 3,121,006. Specific examples of organic resinous materials include polycarbonates, acrylate polymers, vinyl polymers, cellulose polymers, polyesters, polysiloxanes, polyamides, polyurethanes and epoxies as well as block, random or alternating copolymers thereof. Preferred electrically inactive binders are comprised of polycarbonate resins having a molecular weight of from 20,000 to 100,000 with a molecular weight of from 50,000 to 100,000 being particularly preferred. Generally, the resinous binder contains from 10 to 75 percent by weight of the active material corresponding to the foregoing formula, and preferably from 35 percent to 50 percent of this material. In addition, there can be included in the photoresponsive members of the present invention other layers such as a charge blocking layer selected from e.g. polysiloxane, polyamide, polyvinyl butyral, anodized oxide and metal oxide. The thickness of the blocking layer may vary from 0.01 µm (micron) to 5 µm (microns).

Also, included within the scope of the present invention are methods of imaging and printing with the photoresponsive devices illustrated herein. These methods generally involve the formation of an electrostatic latent image on the imaging member, followed by developing the image with a toner composition, subsequently transferring the image to a suitable substrate, and permanently affixing the image thereto. In those environments wherein the device is to be used in a printing mode, the imaging method involves the same steps with the exception that the exposure step can be accomplished with a laser device or image bar.

The invention will now be described in detail with reference to specific preferred embodiments thereof. All parts and percentages are by weight unless otherwise indicated.

### EXAMPLE I

### Synthesis Of AlphaTitanyl Phthalocyanine:

To a three-necked round flask, fitted with a condenser, mechanical stirrer and thermometer was added 14.5 grams of diiminoisoindolene (Aldrich Chemical Company) and 150 milliliters of N-methylpyrrolidone. The mixture was stirred at room temperature under an inert atmosphere of dry argon while 8.85 milliliters of titanium tetra-n-butoxide (Aldrich) was added dropwise over about 5 minutes. The mixture was then stirred and warmed to reflux and maintained at the reflux temperature (about 200°C) for 2 hours.

The resultant black suspension was allowed to cool to about 160°C then was filtered through a 350 milliliter medium porosity sintered glass filter funnel which had been preheated to about 155°C with boiling dimethylformamide (DMF). The solid was washed in the funnel with three 250 milliliter portions of boiling DMF until the filtrate became a light blue-green color. The product was washed again with 250 milliliters of boiling DMF by redispersion of the pigment in the funnel. It was then washed with 100 milliliters of cold DMF then with two 50 milliliter portions of methanol and was dried at 70°C for 20 hours. The product (9.8 grams) of dark blue shiny solid had the following elemental analysis: C, 66.56; H, 2.16; N, 20.17; Ash, 14.15 as compared to the calculated values for alpha titanyl phthalocyanine (C₃₂H₁₆N₈OTi): C, 66.67; H, 2.80; N, 19.44; Ash, 13.86.

### EXAMPLE II

### Synthesis of Alpha Titanyl Phthalocyanine:

The above pigment was prepared by repeating the process of Example I except that 4.74 grams of titanium tetrachloride (Aldrich) was used instead of titanium tetrabutoxide and the reaction mixture was heated at reflux for 6 hours rather than 2 hours. The product, 5.2 grams of shiny blue crystals, had the following elemental analysis: C, 66.77; H, 2.44; N, 19.95; Cl, 0.093; Ash, 13.94. Calculated values for titanyl phthalocyanine are: C, 66.67; H, 2.80; N, 19.44; Cl, 0; Ash, 13.86.

### EXAMPLE III

A photoresponsive imaging member was prepared by providing a titanium metallized Mylar substrate in a thickness of 75 µm (microns)with a DuPont 49,000 polyester adhesive layer thereon in a thickness of 0.05 µm (micron), and depositing thereover in a Balzers vacuum coater a photogenerating layer of the titanyl phthalocyanine obtained by the process of Example I at a final thickness of 0.10 µm (micron). The vacuum coater was evacuated to a pressure of 10⁻⁵ to 10⁻⁶ mbar and the photogenerator pigment was electrically heated in a tantalum boat by a current of 47 amperes. Also, the substrate was situated at 20 centimeters from the boat, and the photogenerator layer was deposited at a rate of about 4 Angstroms/second.

The optical absorption spectrum of the evaporated TiOPc photogenerator layer coated is shown in Figure 2, Line A. It possesses a prominent peak at 740 ± 20 nanometers and a shoulder at a lower wavelength.

Thereafter, the above photogenerating layer was overcoated with an amine charge transport layer prepared as follows: A transport layer solution was prepared by mixing 4.15 grams of Makrolon, a polycarbonate resin, 2.20 grams of N,N'-diphenyl-N,N'-bis(3-methylphenyl)-1,1'-biphenyl-4,4'-diamine and 41 grams of methylene chloride in an amber bottle. The resulting solution was then coated on top of the above photogenerating layer using a multiple clearance film applicator (10 mils wet gap thickness). The resulting member was then dried in a forced air oven at 135°C for 20 minutes and the transport layer had a final thickness of about 20 µm (microns).

The optical absorption of evaporated TiOPc coated with the above transport layer is shown in Figure 2, Line B. The TiOPc has been converted to a new polymorphic form gamma titanyl phthalocyanine exhibiting absorption peaks at 660 ±20 nanometers and 760 ±20 nanometers.

### EXAMPLE IV

The xerographic electrical properties of the photoresponsive member of Example III were determined by electrostatically charging the surface thereof with a corona discharge source until the surface potential, as measured by a capacitively coupled probe attached to an electrometer, attained an initial dark value Vₒ of -800 volts. After resting for 0.5 second in the dark, the charged member reached a surface potential of V_{ddp}, dark development potential. The member was then exposed to light from a filtered Xenon lamp. A reduction in surface potential from V_{ddp} to a background potential V_{bg} due to photodischarge effect was observed. The dark decay in volts/second was calculated as (Vₒ-V_{ddp})/0.5. The percent of photodischarge was calculated as 100 x (V_{ddp}-V_{bg})/V_{ddp}. Half-exposure energy E_{1/2}, the required exposure energy causing reduction of the V_{ddp} to half of its initial value, was determined. The higher the photosensitivity, the smaller its E_{1/2} value. The xerographic electrical results obtained were as follows: dark decay = 24 V/s and E_{1/2} = 4.1-10⁻³ 7/m² (4. erg/cm²)under 780 nanometers exposure.

### EXAMPLE V

Two photoresponsive imaging members were prepared by repeating the procedure of Example III with the exception that the thicknesses of photogenerating layers were 0.20 and 0.30 µm (micron), respectively. Thereafter, the xerographic electricals of the resulting members were determined by repeating the procedure of Example IV with the following results:

| Thickness of Evaporated TiOPc, µm (Microns) | Dark Decay V/s | E_{1/2} in 7/m² (erg/cm²) |
|---|---|---|
| 0.20 | 34 | 3.2·10³ (3.2) |
| 0.30 | 56 | 3.0·10³ (3.0) |
| 0.10 Example III | 24 | 4.1·10³ (4.1) |

The reduction in the E_{1/2} values indicates that the photosensitivity of TiOPc imaging members improved by increasing the thickness of the photogenerator layer as more light is being absorbed by a thicker generator layer. Though the dark decay did increase also, the charge retention properties remained good. Even at the thickest photogenerating layer, for example 0.30 µm (micron), investigated, the loss of surface potential in one second is merely 56 volts, which represents less than 10 percent of initial voltage of the 800 volts.

### EXAMPLE VI

For comparison purposes, vanadyl phthalocyanine (VOPc) was used in fabricating a photoresponsive imaging member following the procedure of Example III. The thickness of the photogenerating layer was kept at 0.10 µm (micron).

The following table summarizes the xerographic results obtained for VOPc and TiOPc imaging members fabricated and tested under identical conditions. The TiOPc has a E_{1/2} which is 1/7 of VOPc's value, and hence exhibits higher photosensitivity than VOPc

| Photogenerator | Dark Decay V/s | E_{1/2} in 7/m² (erg/cm²) |
|---|---|---|
| 0.10 µm (micron) VOPc | 26 | 28.4·10⁻³ (28.4) |
| 0.10 µm (micron) TiOPc, Example III | 24 | 4.1·10⁻³ (4.1) |

## Claims

1. A photoresponsive imaging member comprised of a supporting substrate, a charge generating layer deposited thereon consisting of a vacuum evaporated photogenerator layer of gamma titanyl phthalocyanine of the formula C₃₂H₁₆N₈OTi with two major optical absorption peaks at 660 and 760 nm, and a charge transporting layer deposited on said charge generating layer, wherein the peaks are achieved subsequent to the deposition of said transport layer on said titanyl phthalocyanine layer, wherein the charge transport layer is an aryl amine hole transport layer comprised of molecules of the formula wherein X is selected from the group consisting of halogen atom and alkyl group, dispersed in a resinous binder under the addition of an organic solvent, and wherein the solvent is selected from the group consisting of methylene chloride, chlorobenzene, toluene, cyclohexanone and alcohols.

2. The photoresponsive imaging member in accordance with claim 1 wherein the alcohol is methanol.

3. The photoresponsive imaging member in accordance with claim 1 wherein the supporting substrate is comprised of a conductive metallic or nonmetallic substance, conductive filler loaded plastic, or an insulating polymeric composition overcoated with an electrically conductive layer.

4. The photoresponsive imaging member in accordance with claim 1 wherein the supporting substrate is aluminum or carbon-loaded conductive plastic.

5. The photoresponsive imaging member in accordance with claim 1 wherein the supporting substrate is overcoated with a polymeric adhesive layer.

6. The photoresponsive imaging member in accordance with claim 5 wherein the adhesive layer is a polyester resin.

7. The photoresponsive imaging member in accordance with claim 1 wherein X is selected from (ortho) CH₃, (meta) CH₃, (para) CH₃, (ortho) Cl, (meta) Cl, and (para) Cl.

8. The photoresponsive imaging member in accordance with claim 1 wherein the aryl amine is N,N'-diphenyl-N,N'-bis(3-methylphenyl)-1,1'-biphenyl-4,4'-diamine.

9. The photoresponsive imaging member in accordance with claim 1 wherein the resinous binder is a polycarbonate or polyvinylcarbazole.

10. The photoresponsive imaging member in accordance with claim 1 wherein the titanyl phthalocyanine is dispersed in a resinous binder in an amount of from 5 percent to 95 percent by volume, and the aryl amine hole transport molecules are dispersed in a resinous binder in an amount of from 10 to 75 percent by weight.

11. The photoresponsive imaging member in accordance with claim 10 wherein the resinous binder for the titanyl phthalocyanine is a polyester, a polyvinylcarbazole, polyvinylbutyral, a polycarbonate, or a phenoxy resin; and the resinous binder for the aryl amine hole transport material is a polycarbonate, a polyester, or a vinyl polymer.

12. The photoresponsive imaging member in accordance with claim 1 containing a protective wear resistant layer.

13. The photoresponsive imaging member in accordance with claim 12 wherein the protective layer is selected from a polycarbonate or a polyurethane.

14. The photoresponsive imaging member in accordance with claim 12 wherein the protective layer is comprised of polymer containing abrasive materials.

15. The photoresponsive imaging member in accordance with claim 14 wherein the abrasive materials are selected from the group consisting of silicon dioxide, hydrogenated amorphous carbon, and silicon carbides.

16. The photoresponsive imaging member in accordance with claim 15 wherein the abrasive material is present in an amount of from 1 to 25 weight percent.

17. The photoresponsive imaging member in accordance with claim 1 wherein the solvent dispersion of charge transport molecules in solution coated onto the charge generating layer comprising titanyl phthalocyanine is subsequently dried.

18. The photoresponsive imaging member in accordance with claim 17 wherein drying is accomplished by heating at a temperature of from 100 to 150°C.

19. The photoresponsive imaging member in accordance with claim 18 wherein heating is accomplished for a period of from 1 minute to 120 minutes.

20. The photoresponsive imaging member in accordance with claim 19 wherein heating is accomplished for a period of from 2 minutes to 60 minutes.

21. A method of imaging or printing which comprises forming an elestrostatic latent image on the photoresponsive imaging member of any of claims 1 to 20 accomplishing development thereof with toner particles; subsequently transferring the developed image to a suitable substrate; and permanently affixing the image thereto.

## Patentansprüche

1. Ein photoempfindliches Abbildungselement, umfassend ein Trägersubstrat, eine darauf aufgetragene ladungsbildende Schicht, bestehend aus einer vakuumverdampften photobildenden Schicht aus gamma-Titanylphtalocyanin der Formel C₃₂H₁₆N₈OTi mit zwei ausgeprägten optischen Absorptionsspitzen bei 660 und 760 nm, und eine auf besagter ladungsbildender Schicht aufgetragene ladungstransportierende Schicht, wobei die Spitzen nach dem Auftrag der besagten Transportschicht auf die besagte Titanylphtalocyanin-Schicht ausgebildet werden, wobei die Ladungstransportschicht eine Arylaminlochtransportschicht, umfassend Moleküle der Formel ist, worin X ausgewählt ist aus der Gruppe bestehend aus einem Halogenatom und einer Alkylgruppe, dispergiert in einem harzhaltigen Bindemittel unter dem Zusatz eines organischen Lösungsmittels und wobei das Lösungsmittel ausgewählt ist aus der Gruppe bestehend aus Methylenchlorid, Chlorbenzol, Toluol, Cyclohexanon und Alkoholen.

2. Das photoempfindliche Abbildungselement gemäß Anspruch 1, wobei der Alkohol Methanol ist.

3. Das photoempfindliche Abbildungselement gemäß Anspruch 1, wobei das Trägersubstrat eine leitende metallische oder nicht-metallische Verbindung, mit leitendem Füllmaterial beladenen Kunststoff oder eine mit einer elektrisch leitenden Schicht überzogene isolierende polymere Zusammensetzung umfaßt.

4. Das photoempfindliche Abbildungselement gemäß Anspruch 1, wobei das Trägersubstrat Aluminium oder Kohlenstoff beladener leitender Kunststoff ist.

5. Das photoempfindliche Abbildungselement gemäß Anspruch 1, wobei das Trägersubstrat mit einer polymeren Klebeschicht überzogen ist.

6. Das photoempfindliche Abbildungselement gemäß Anspruch 5, wobei die Klebeschicht ein Polyesterharz ist.

7. Das photoempfindliche Abbildungselement gemäß Anspruch 1, wobei X ausgewählt ist aus (ortho) CH₃, (meta) CH₃, (para) CH₃, (ortho) Cl, (meta) Cl und (para) Cl.

8. Das photoempfindliche Abbildungselement gemäß Anspruch 1, wobei das Arylamin N, N'-Diphenyl-N, N'-bis (3-methylphenyl)-1, 1'-biphenyl-4, 4'-diamin ist.

9. Das photoempfindliche Abbildungselement gemäß Anspruch 1, wobei das harzhaltige Bindemittel ein Polycarbonat oder Polyvinylcarbazol ist.

10. Das photoempfindliche Abbildungselement gemäß Anspruch 1, wobei das Titanylphthalocyanin in einem harzhaltigen Bindemittel in einer Menge von 5 Prozent bis 95 Volumenprozent dispergiert ist und die Arylaminlochtransportmoleküle in einem harzhaltigen Bindemittel in einer Menge von 10 bis 75 Gewichtsprozent dispergiert sind.

11. Das photoempfindliche Abbildungselement gemäß Anspruch 10, wobei das harzhaltige Bindemittel für das Titanylphthalocyanin ein Polyester, ein Polyvinylcarbazol, Polyvinylbutyral, ein Polycarbonat oder ein Phenoxyharz ist; und das harzhaltige Bindemittel für das Arylaminlochtransportmaterial ein Polycarbonat, ein Polyester oder ein Vinylpolymer ist.

12. Das photoempfindliche Abbildungselement gemäß Anspruch 1, enthaltend eine schützende abnutzungsresistente Schicht.

13. Das photoempfindliche Abbildungselement gemäß Anspruch 12, wobei die schützende Schicht ausgewählt ist aus einem Polycarbonat oder einem Polyurethan.

14. Das photoempfindliche Abbildungselement gemäß Anspruch 12, wobei die schützende Schicht aus einem abreibende Materialien enthaltenden Polymer besteht.

15. Das photoempfindliche Abbildungselement gemäß Anspruch 14, wobei das abreibende Material ausgewählt ist aus der Gruppe bestehend aus Siliziumdioxid, hydrogeniertem amorphen Kohlenstoff und Siliziumcarbiden.

16. Das photoempfindliche Abbildungselement gemäß Anspruch 15, wobei das abreibende Material in einer Menge von 1 bis 25 Gewichtsprozent vorhanden ist.

17. Das photoempfindliche Abbildungselement gemäß Anspruch 1, wobei die Lösungsmitteldispersion der ladungstransportierenden Moleküle in Lösung, die auf die Titanylphthalocyanin enthaltende ladungsbildende Schicht aufgetragen wird, anschließend getrocknet wird.

18. Das photoempfindliche Abbildungselement gemäß Anspruch 17, wobei die Trocknung durch Erhitzen auf eine Temperatur von 100 bis 150°C durchgeführt wird.

19. Das photoempfindliche Abbildungselement gemäß Anspruch 18, wobei das Erhitzen für einen Zeitraum von 1 Minute bis 120 Minuten durchgeführt wird.

20. Das photoempfindliche Abbildungselement gemäß Anspruch 19, wobei das Erhitzen für einen Zeitraum von 2 Minuten bis 60 Minuten durchgeführt wird.

21. Ein Verfahren zur Abbildung oder zum Drucken, welches das Ausbilden einer elektrostatischen latenten Abbildung auf dem photoempfindlichen Abbildungselement von einem der Ansprüche 1 bis 20, das Durchführen der Entwicklung davon mit Tonerpartikeln; das anschließende Überführen der entwickelten Abbildung auf ein geeignetes Substrat; und die permanente Fixierung der Abbildung darauf, umfaßt.

## Revendications

1. Elément de formation d'image photosensible constitué d'un substrat de support, d'une couche de génération de charges déposée sur celui-ci constituée d'une couche de générateur photoélectrique évaporée sous vide de phtalocyanine de titanyle gamma de formule C₃₂H₁₆N₈OTi présentant deux pics d'absorption optique principaux à 660 et à 760 nanomètres, et d'une couche de transport de charges déposée sur ladite couche de génération de charges, dans lequel les pics sont
obtenus à la suite du dépôt de ladite couche de transport sur ladite couche de phtalocyanine de titanyle, dans lequel la couche de transport de charges est une couche d'arylamine de transport de trous constituée de molécules de la formule dans laquelle X est choisi parmi le groupe constitué d'un atome halogène et d'un groupement alkyle, dispersées dans un liant résineux sous l'addition d'un solvant organique, et dans lequel le solvant est choisi parmi le groupe constitué du chlorure de méthylène, du chlorobenzène, du toluène, de la cyclohexanone et d'alcools.

2. Elément de formation d'image photosensible selon la revendication 1, dans lequel l'alcool est le méthanol.

3. Elément de formation d'image photosensible selon la revendication 1, dans lequel le substrat de support est constitué d'une substance conductrice métallique ou non métallique, d'une matière plastique conductrice garnie d'une charge ou d'une composition polymère isolante revêtue d'une couche électroconductrice.

4. Elément de formation d'image photosensible selon la revendication 1, dans lequel le substrat de support est de l'aluminium ou une matière plastique conductrice chargée en carbone.

5. Elément de formation d'image photosensible selon la revendication 1, dans lequel le substrat de support est revêtu d'une couche adhésive polymère.

6. Elément de formation d'image photosensible selon la revendication 5, dans lequel la couche adhésive est une résine de polyester.

7. Elément de formation d'image photosensible selon la revendication 1, dans lequel X est choisi parmi CH₃ (en ortho), CH₃ (en métal, CH₃ (en para), Cl (en ortho), Cl (en méta) et Cl (en para).

8. Elément de formation d'image photosensible selon la revendication 1, dans lequel l'arylamine est la N,N'-diphényl-N,N'-bis(3-méthylphényl)-1,1'-biphényl-4,4'-diamine.

9. Elément de formation d'image photosensible selon la revendication 1, dans lequel le liant résineux est un polycarbonate ou un polyvinylcarbazole.

10. Elément de formation d'image photosensible selon la revendication 1, dans lequel la phtalocyanine de titanyle est dispersée dans un liant résineux dans une proportion de 5 pour cent à 95 pour cent en volume, et les molécules d'arylamines de transport de trous sont dispersées dans un liant résineux dans une proportion de 10 à 75 pour cent en poids.

11. Elément de formation d'image photosensible selon la revendication 10, dans lequel le liant résineux pour la phtalocyanine de titanyle est un polyester, un polyvinylcarbazole, un polyvinylbutyral, un polycarbonate, ou une résine phénoxy, et le liant résineux pour le matériau d'arylamine de transport de trous est un polycarbonate, un polyester ou un polymère vinylique.

12. Elément de formation d'image photosensible selon la revendication 1, contenant une couche protectrice résistante à l'usure.

13. Elément de formation d'image photosensible selon la revendication 12, dans lequel la couche protectrice est choisie parmi un polycarbonate ou un polyuréthane.

14. Elément de formation d'image photosensible selon la revendication 12, dans lequel la couche protectrice est constituée d'un polymère contenant des matériaux abrasifs.

15. Elément de formation d'image photosensible selon la revendication 14, dans lequel les matériaux abrasifs sont choisis parmi le groupe constitué de dioxyde de silicium, de carbone amorphe hydrogéné et de carbures de silicium.

16. Elément de formation d'image photosensible selon la revendication 15, dans lequel le matériau abrasif est présent dans une proportion de 1 à 25 pour cent en poids.

17. Elément de formation d'image photosensible selon la revendication 1, dans lequel la dispersion dans un solvant des molécules de transport de charges en solution appliquées sur la couche de génération de charges comprenant de la phtalocyanine de titanyle est ensuite séchée.

18. Elément de formation d'image photosensible selon la revendication 17, dans lequel le séchage est réalisé par chauffage à une température de 100 à 150 °C.

19. Elément de formation d'image photosensible selon la revendication 18, dans lequel le chauffage est réalisé pendant une période de 1 minute à 120 minutes.

20. Elément de formation d'image photosensible selon la revendication 19, dans lequel le chauffage est réalisé pendant une période de 2 minutes à 60 minutes.

21. Procédé de formation d'image ou d'impression qui comprend la formation d'une image latente électrostatique sur l'élément de formation d'image photosensible selon l'une quelconque des revendications 1 à 20, en réalisant le développement de celle-ci avec des particules de toner, le transfert ensuite de l'image développée sur un substrat approprié, et le fixage de façon permanente de l'image sur celui-ci.
